

Jan. 14, 1958

M. SALO ET AL

2,819,983

WOOD FINISHING LACQUER SYSTEMS

Filed Feb. 1, 1954



MARTIN SALO  
GERARD J. CLARKE  
JOHN GALLAGHER  
INVENTORS

BY *Daniel J. Mayne*,  
*Henry E. Byers*  
ATTORNEYS

2,819,983

## WOOD FINISHING LACQUER SYSTEMS

Martin Salo, Gerard J. Clarke, and John F. Gallagher,  
Rochester, N. Y., assignors to Eastman Kodak Company,  
Rochester, N. Y., a corporation of New Jersey

Application February 1, 1954, Serial No. 407,581

2 Claims. (Cl. 117—73)

This invention relates to ternary wood finishing lacquer systems, particularly systems based on cellulose acetate butyrate.

Hitherto, lacquers used in wood finishing have generally been produced with nitrocellulose as a base, particularly the one-half second and one-quarter second types. However, cellulose nitrate has certain limitations with respect to heat and ultraviolet light stability. Attempts have been made to substitute various cellulosic esters for cellulose nitrate without noticeable success. In some adaptations, cellulose acetate has been found unsuitable because of its incompatibility with most natural, and especially with most synthetic resins, necessary ingredients of a lacquer satisfactory for general use. For instance, cellulose acetate is incompatible with various polybasic acid-polyhydric alcohol resins, phenol-formaldehyde resins, vinyl acetate resins, etc., all of which are valuable types of lacquer resins, in the proportions necessary for the formulation of a satisfactory lacquer. Cellulose acetate butyrate is compatible with synthetic resins, but has been found unsuitable for coating over commonly used sealers and fillers. Consequently, there has been a need for a system of lacquering coats which are compatible with each other, and which form a unitary system. This invention meets that need in that it provides three successive coatings, each performing a specific task, but each inseparably united with each other due to the particular affinity for the other coatings.

One of the objects of this invention is to provide a high gloss wood finishing lacquer. Another object of this invention is to provide a ternary wood finishing system having a cellulose acetate butyrate base. A further object of this invention is to provide a brushing or spraying lacquer system containing cellulose acetate butyrate and compatible ingredients to form a hard finish wood surface coating.

A normal system for coating wood consists of three or more successive coats in which the first three perform specific functions. A filler coat which contains some filler material which fills the pores of the wood to provide a smooth surface is ordinarily first applied over the sanded surface. In conventional type fillers, linseed oil is a predominant vehicle. Consequently, it has been found that cellulose acetate butyrate lacquers applied over this type of filler may have poor adhesion and inferior appearance due possibly to the migration of the incompatible linseed oil into the sealer and topcoats. The fillers, provided in this invention, contain cellulose acetate butyrate, a large amount of inorganic material such as talc, in low-cost solvent mixtures such as ones containing a large proportion of turpentine and dipentene.

A sanding sealer is next applied to the surface following the filling operation and sanded or buffed to a fine finish. One, two, or more coats may be applied depending upon the finish desired. This coating must be easily sandable to a fine finish and adherent both to the filled surface and top coats. The sealer must also be successfully flexible to withstand the dimensional changes occur-

ring in the wood caused by aging and normal fluctuation in temperature and humidity. The sealers of this invention, based on cellulose acetate butyrate, have worked out successfully as sanding sealers having good adhesion to the corresponding fillers and to cellulose acetate butyrate top coat lacquers.

Top coats are applied following the buffing of the sealer coat. The top coats of this invention are based upon cellulose acetate butyrate and have good affinity and adhesion for the preceding cellulose acetate butyrate coatings used for sealer and filler. However, the main feature of this invention is in the proper integration of the top coat lacquer with corresponding fillers and sealers to obtain a high grade high gloss finish.

The attached diagrammatic drawing illustrates our integrated 3-coat system for wood using a cellulose acetate butyrate filler, a cellulose acetate butyrate sealer and a cellulose acetate butyrate top coat.

The following tables give formulas which have been found satisfactory for the respective coatings.

TABLE I  
Wood grain fillers

|                                                        | 1    | 2    | 3    | 4  | 5  |
|--------------------------------------------------------|------|------|------|----|----|
| Cellulose acetate butyrate (about 37% butyryl) percent | 1.4  | 1.4  | 2.3  | 6  | 6  |
| Aropiaz 905 do                                         | 9.6  | 9.6  | —    | —  | —  |
| Aropiaz 945 do                                         | 2.4  | 2.4  | —    | —  | —  |
| Talc do                                                | 38.5 | 38.5 | —    | —  | —  |
| Vinylite VMCH do                                       | —    | —    | 3.4  | —  | —  |
| Santolite MHP do                                       | —    | —    | —    | 9  | —  |
| Petrex 37 do                                           | —    | —    | —    | —  | 9  |
| Asbestine X do                                         | —    | —    | 5.7  | 15 | 15 |
| Percent solvent                                        | 48.1 | 48.1 | 88.6 | 70 | 70 |
| Type of solvent                                        | 1    | 2    | 3    | 4  | 4  |

### SOLVENTS

1=50% turpentine, 22.2% butyl acetate, 13.4% butyl alcohol, 3.3% butyl Cellosolve, 11.1% #1 ethyl alcohol.

2=50% dipentene, 22.2% butyl acetate, 13.4% butyl alcohol, 3.3% butyl Cellosolve, 11.1% #1 ethyl alcohol.

3=47.5% isobutyl acetate, 10.9% n butyl alcohol, 13.0% toluene, 28.6% methyl isobutyl ketone.

4=33.3% diacetone alcohol, 33.3% butyl acetate, 15.2% n butyl alcohol, 18.2% toluene.

The solvent to solid ratio in the above formulations may vary from 1:1 to 9:1. The composition of the solid constituents includes from 2 to 30% cellulose acetate butyrate which has above about 35% butyryl content with an intrinsic viscosity of .5 to 2.0 in acetone. An adhesive resin, selected from a non-oxidizing pure short oil alkyd, a semi-oxidizing pure medium oil alkyd, a vinyl chloride acetate-dibasic acid copolymer, an aryl sulfonamide-formaldehyde condensate, or a terpine acid-rosin coester, which is added to the filler, may range from 10 to 30%. The mineral filler which may be Asbestine X or talc can vary in an amount from 30 to 70%. Solvents are low cost compatible organic compounds suitable for spray or brush application.

TABLE II  
Sanding sealers

|                                                | 1                   | 2                   | 3                   | 4                 | 5                    | 6                    | 7                  |
|------------------------------------------------|---------------------|---------------------|---------------------|-------------------|----------------------|----------------------|--------------------|
|                                                | Per-<br>cent<br>4.5 | Per-<br>cent<br>4.5 | Per-<br>cent<br>6.0 | Per-<br>cent<br>8 | Per-<br>cent<br>13.0 | Per-<br>cent<br>13.0 | Per-<br>cent<br>14 |
| Cellulose acetate butyrate (about 37% butyryl) |                     |                     |                     |                   |                      |                      |                    |
| Arochem 404                                    | 24.1                |                     |                     |                   |                      |                      |                    |
| Arochem 545                                    |                     | 24.1                | 14.0                | 12                | 6.0                  | 7.0                  | —                  |
| Diocetyl phthalate                             |                     |                     |                     |                   | 1.0                  | —                    | —                  |
| Solvent <sup>1</sup>                           | 71.4                | 71.4                | 80                  | 80                | 80                   | 80                   | —                  |
| Solvent <sup>2</sup>                           |                     |                     |                     |                   |                      |                      | 86                 |

<sup>1</sup> Solvent=20% xylene, 30% toluene, 10% butyl alcohol, 20% ethanol 20% butyl acetate.

<sup>2</sup> Solvent=24.5% acetone, 23.2% butyl acetate, 23.2% butyl Cellosolve, 10.5% No. 1 ethanol, 18.6% toluene.

The solvent to solid ratio in the sanding sealer formulations may be from 1:1 to 5:1. The composition of the solid constituents which we have found operative includes from 10 to 100% cellulose acetate butyrate having above about 35% butyryl content and an intrinsic viscosity of from .5 to 2.0 in acetone. The hard adhesive resin, selected from rosin modified condensates or rosin modified maleic acid resins, may vary from 0 to 90%. A plasticizer, such as diethyl phthalate, may be in an amount of 0 to 10%. The solvents which are low cost organic compounds may be substituted with other suitable compositions which are compatible with the materials to be sprayed or brushed.

TABLE III  
Top coats

| Composition of solids (dry basis)              | 1   | 2   | 3    | 4    | 5   | 6   | 7   | 8    | 9    | 10  |
|------------------------------------------------|-----|-----|------|------|-----|-----|-----|------|------|-----|
| Cellulose acetate butyrate (about 37% butyryl) | 90  | 85  | 56.4 | 86.3 | 90  | 85  | 85  | 45.8 | 80.0 | 50  |
| Dammar                                         | 10  | 15  | 8.9  | 5.3  | 10  | 15  | 15  |      | 15.0 | 50  |
| Synthe copal                                   |     |     | 13.7 |      |     |     |     | 2.6  |      |     |
| Aroplaz 1130                                   |     |     |      |      |     |     |     | 33.0 |      |     |
| Arochem 404                                    |     |     |      |      |     |     |     | 9.3  |      |     |
| Tegiac 15                                      |     |     |      |      |     |     |     |      |      | 10  |
| Aroplaz 905T                                   |     |     |      |      |     |     |     |      |      | 40  |
| Bakelite BJ-16580                              |     |     |      |      |     |     |     | 9.3  |      |     |
| Dibutyl phthalate                              |     |     | 21.0 | 8.4  |     |     |     |      | 5    |     |
| Diethyl phthalate                              |     |     |      |      |     |     |     |      |      | 3   |
| Solvent                                        | 1   | 1   | 1    | 1    | 1   | 1   | 1   | 1    | 2    |     |
| Solvent-Solid ratio                            | 9:1 | 9:1 | 9:1  | 9:1  | 9:1 | 9:1 | 9:1 | 9:1  | 9:1  | 9:1 |

<sup>1</sup> Solvent 1—55% toluene, 10% #1 ethyl alcohol, 32% butyl acetate, 3% Cellosolve acetate.  
Solvent 2—20% xylene, 30% butyl acetate, 15% #1 ethyl alcohol, 25% toluene, 10% butyl alcohol.  
Solvent 3—20% xylene, 35% butyl acetate, 35% toluene, 10% butanol.

The solvent to solid ratio in the top coat formulations may vary from 10:1 to 3:1. The composition of the solid

amount of rosin. Copal is a common ester gum which may be synthesized by the reaction of glycerol with rosin.

TABLE IV

| Resin         | Resin type                                        | Type of oil | Oil content | Phthalic acid content | Acid No. |
|---------------|---------------------------------------------------|-------------|-------------|-----------------------|----------|
| Aroplaz 905   | Non-oxidizing, pure short oil alkyd               | Cocoanut    | Percent     | Percent               | 6-12     |
| Aroplaz 945   | Semi-oxidizing, pure medium oil alkyd             | Soya-castor | 51          | 34.5                  | 4-7      |
| Aroplaz 1130  | Oxidizing, short oil alkyd                        | Soya        | 40          | 38                    | 4-8      |
| Arochem 404   | Rosin modified condensate                         |             |             |                       | 280-300  |
| Arochem 545   | Rosin modified maleic                             |             |             |                       | 25-35    |
| Tegiac 15     | Rosin modified alkyd                              |             |             |                       |          |
| Synthe copal  | Ester gum (ester of glycerol and rosin)           |             |             |                       | 6-8      |
| Vinylite VMCH | Vinyl chloride-acetate resin with .7-.8% carboxyl |             |             |                       |          |
| Santolite MHP | Aryl sulfonamide formaldehyde condensate          |             |             |                       |          |
| Petrex 37     | Terpine acid-rosin coester                        |             |             |                       | 30       |
| Dammar        | Natural resin                                     |             |             |                       | 20-30    |
| Asbestine X   | Magnesium silicate                                |             |             |                       |          |
| Tale          | do                                                |             |             |                       |          |

constituents includes cellulose acetate butyrate from 40 to 90% having above about 35% butyryl content and an intrinsic viscosity of .5 to 2.0 in acetone. The intrinsic viscosity is determined by measuring the flow rate of a solution of 0.25 g. of the test composition made up to 100 cc. with acetone. A measure of the flow time at 25° C. gives the relative viscosity. Relative viscosity

$$(n_r) = \frac{\text{flow time for solution}}{\text{flow time for solvent}}$$

Intrinsic viscosity ( $n_r$ ) is equal to  $9.21 \log (n_r)$ . The hard adhesive resins which may be added in an amount of from 10 to 30% are selected from Dammar (natural resin), ester gum, oxidizing short oil alkyd resins, rosin modified condensates, and rosin modified alkyd and phenolic resins. A plasticizer, dibutyl phthalate or diethyl phthalate or a soft resin such as a non-oxidizing pure oil alkyd resin is added in an amount of from 10 to 30%. The solvent is a mixture of low cost organic solvents as indicated above, but it is obvious that these specific components may be substituted by others which are compatible and which are equally effective.

The following table lists commercially available ma-

terials with their trade names with a description of the type of material as well as additional information. By alkyd resins we mean resins which are made by condensing glycerol and phthalic anhydride plus an oil which may be cocoanut oil or the like. Non-oxidizing pure short oil alkyd resins include those in which the oil is castor oil, cocoanut oil or a similar oil. Semi-oxidizing pure medium oil alkyd resins use soya oil in admixture with castor or cocoanut oil. Oxidizing short oil alkyd resins use soya, linseed, dehydrated castor, or tung oils. Rosin modified maleic resin comprises a rosin maleic acid condensate. A rosin modified alkyd resin is a glycerol-phthalic anhydride product hardened by adding an

The above compositions might be used separately if compatible corresponding coatings were also used. However, the preferred embodiment of this invention is the ternary system. Only through the successive coating of the filler, sealer and topcoat is the integrated coating formed. This integrated coating has the basic characteristics which make it unique in the art. The filler has unusually good adhesion to wood yet has affinity for the sealer. The sealer has exceptional sanding and buffing characteristics and is particularly unique in its bonding ability for both the filler and top coat. The top coat in addition to forming the third unit in this coating also has excellent brushing characteristics, and provides a good gloss.

We claim:

1. An article comprising a wooden structure having thereon a ternary wood-finishing lacquer system having a cellulose acetate butyrate base in each of the three components, a filler coat comprising 2-30 parts cellulose acetate butyrate, magnesium silicate and 10-30 parts of an adhesive resin selected from the class consisting of non-oxidizing pure short-oil alkyd resins, semioxidizing pure medium-oil alkyd resins, vinyl chloride-acetate-dibasic

acid copolymers, aryl sulfonamide-formaldehyde condensate, and terpine acetate-rosin-coester, a sanding sealer comprising 10-100 parts of cellulose acetate butyrate, 90-10 parts of a rosin maleic acid condensate, and a plasticizer, a top coat comprising 40-90 parts cellulose acetate butyrate, a plasticizer selected from the class consisting of dibutyl phthalate and dioctyl phthalate, and 10-30 parts of a hard resin selected from the class consisting of Dammar, ester gum, an oxidizing short-oil alkyd resin and a rosin-modified alkyd phenolic resin.

2. An article comprising a wooden structure having thereon a ternary wood-finishing lacquer system having a cellulose acetate butyrate base in each of the three components, the filler coat comprising from 2-30 parts cellulose acetate butyrate, magnesium silicate and 10-30 parts of an adhesive resin selected from the class consisting of nonoxidizing pure short-oil alkyd resin, semioxidizing pure medium-oil alkyd resins, vinyl chloride-acetate-dibasic acid copolymers, aryl sulfonamide-formaldehyde condensates and terpine acid-rosin coesters, a sanding sealer comprising 10-100 parts cellulose acetate butyrate, from 0-90 parts of a rosin-modified maleic resin and from 0-10 parts

of a plasticizer, a top coat comprising 40-90 parts cellulose acetate butyrate, from 10-30 parts of a hard adhesive resin selected from the class consisting of Dammar, ester gum, an oxidizing short-oil alkyd resin and a rosin-modified alkyd phenolic resin and from 10-30 parts of a plasticizer selected from the class consisting of dibutyl phthalate and dioctyl phthalate.

## References Cited in the file of this patent

10

## UNITED STATES PATENTS

|           |             |               |
|-----------|-------------|---------------|
| 2,113,305 | Malm        | Apr. 5, 1938  |
| 2,186,454 | Gloor       | Jan. 9, 1940  |
| 2,324,098 | Malm et al. | July 13, 1943 |
| 2,375,753 | Clare       | May 15, 1945  |
| 2,379,974 | Little      | July 10, 1945 |
| 2,572,252 | Erasmus     | Oct. 23, 1951 |

## OTHER REFERENCES

20 Wampler: Organic Finishing, vol. 10, issue 11, pp. 17-19, November 1949.